

Nov. 30, 1937.

O. E. HARDER

2,100,314

LINER FOR BEARINGS

Filed Nov. 5, 1934



INVENTOR.  
Oscar E. Harder

BY  
Locher & Mahoney  
ATTORNEYS.

## UNITED STATES PATENT OFFICE

2,100,314

## LINER FOR BEARINGS

Oscar E. Harder, Columbus, Ohio, assignor, by  
mesne assignments, to Federal-Mogul Corporation,  
Detroit, Mich., a corporation of Michigan

Application November 5, 1934, Serial No. 751,546

10 Claims. (Cl. 308—242)

My invention relates to liners for bearings. It has to do particularly with a novel liner for bearings for rotating shafts designed to operate under heavy loads and at high speeds, although 5 it is not necessarily limited thereto.

The use of relatively soft metals or alloys as liners for bearings is old. One purpose of such use is to provide, as a support for the shaft, a contacting surface which will adequately support a hardened steel shaft or the like and, at the same time, which will avoid scoring or seriously abrading the shaft as it rotates within the bearing.

The metals which have been most extensively used for this purpose may be generally classed as tin-base and lead-base alloys. The tin-base alloys are mainly composed of tin but usually contain substantial percentages of copper and antimony, increasing in hardness as the contents of copper and antimony are increased. The lead-base alloys are mainly composed of lead, but usually contain significant percentages of one or more of the metals, antimony, tin and copper, which generally serve to harden the alloy.

In addition to the tin-base and lead-base alloys, other alloys are, to a lesser extent, in use as bearing linings. These include alloys consisting of cadmium, zinc and antimony, alloys of 30 cadmium and nickel, and alloys of cadmium and copper. Lead, hardened with one or more alkali metals or alkaline earth metals, such as sodium, calcium, barium and lithium, has also been used as a bearing lining.

It is more or less generally recognized in the art that alloys which are desirable as lining materials for bearings should be composed of harder particles embedded in a relatively soft matrix. The theory is that the harder particles 40 serve to make the contact and directly carry the load, while the softer matrix permits the lining material to conform to the shape of the moving member or shaft.

My invention contemplates the production of 45 a lining material for bearings wherein the primary ingredients are cadmium and silver alloyed to form a relatively soft but tough matrix. Such an alloy may be formed either by fusion and casting of the alloy metals or by electrodeposition. The proportions of these metals may vary 50 but I prefer that the cadmium be the base metal and that the silver be introduced in relatively small percentages. I preferably use from .10 to 15 per cent of silver, with the balance of the 55 alloy cadmium.

This application is a continuation in part of my application, Serial No. 732,181, filed June 23, 1934, and my application, Serial No. 743,874, filed September 13, 1934.

Under preferred conditions, where my bearing material is to take the form of a binary alloy of cadmium and silver, I preferably use in excess of 3 per cent silver, since my tests have indicated that silver goes into solid solution with cadmium up to approximately 3 per cent of the 10 silver, while the excess over and above the 3 per cent of silver will form intermetallic compounds of silver and cadmium which are dispersed throughout the alloy as small hard particles. In this way, I am able to produce a lining material 15 for bearings wherein the solid solution of cadmium and silver form the relatively soft but tough matrix, while the intermetallic compounds of silver and cadmium which are dispersed throughout this matrix as small hard particles 20 serve to make the contact and directly carry the load.

By way of illustration, the accompanying drawing shows a photomicrograph, taken at 1000 diameters, wherein the alloy contains 3 per cent 25 by weight of silver and the balance cadmium. From this drawing, it will be seen that the small hard particles of intermetallic compound appear as white spots 5, which are embedded in a matrix that is apparently made up of a cored structure.

In studying lining materials made in accordance with my invention, I have prepared alloys of cadmium and silver containing varying silver contents up to 10 per cent. These alloys were 35 prepared by fusion and casting and their hardness and microstructures were determined. The data obtained in this connection showed that the cast alloys increased in hardness as the silver content increased, and hardnesses of 38 to 55 40 Brinell (500 kg. load) were obtained. The study of these alloys further showed that in the compositions containing approximately 3 per cent of silver and over the microstructure consisted of two phases. These phases apparently comprised the soft matrix formed by solid solution of silver in cadmium and a number of relatively 45 small hard particles dispersed throughout such soft matrix. The amount of harder particles increased as the silver content increased.

By electrodeposition, with the use of independent soluble anodes of cadmium and silver and by the use of an alkaline cyanide bath, I have deposited bearing lining alloys containing from 1.72 to 20 per cent of silver. At the present time, 55

for most purposes, I consider that a binary alloy containing 3 per cent of silver is somewhat too soft and that an alloy containing more than 15 per cent of silver is inclined to be brittle and costly. However, for some classes of bearing service, an alloy containing as low as .10 per cent of silver may be suitable and is within the scope of my invention. As a matter of fact, the presence of even as little as .10 per cent of silver in the alloy improves the casting qualities of the cadmium, making it less susceptible to oxidation and drossing. Likewise, even a small percentage of added silver increases the fluidity, raises the melting point and improves the strength and hardness of the alloy.

Binary alloys which I have made by electrodeposition show substantially the same microconstituents as cadmium-silver alloys prepared by fusion and casting, although the shape and distribution may be somewhat different. Likewise, the grain structure is somewhat finer.

I have determined the hardness of cadmium-silver alloys in the as-cast condition, because it is not convenient to make hardness tests on thin plates of these alloys as formed by electrodeposition. In series of tests to determine the effect of adding silver to cadmium on the hardness at room temperature and at elevated temperatures, the following results were obtained:

30 *Brinell hardness at room and elevated temperature of some cadmium base alloys*

| 35 | Composition |         | Temperature |         |         |
|----|-------------|---------|-------------|---------|---------|
|    | Cadmium     | Silver  | Room        | 212° F. | 390° F. |
|    | Percent     | Percent |             |         |         |
| 40 | 100.00      | 1.07    | 23.0        | 18.2    | 7.1     |
|    | 98.93       | 2.10    | 29.8        | 18.6    | 7.4     |
|    | 97.90       | 2.01    | 34.4        | 20.9    | 9.5     |
|    | 97.09       | 5.06    | 36.2        | 22.8    | 10.0    |
|    | 94.94       |         | 40.2        |         |         |

The following table shows the hardness of alloys containing 6.4 per cent and 8.0 per cent of silver, respectively, at temperatures of 70°, 350°, and 450° F. For comparison purposes, hardness tests on a babbitt containing 85 per cent tin, 7.5 per cent copper, and 7.5 per cent antimony have 50 been included:

55 *Comparison of hardness of cadmium-silver alloys with babbitt*

| 60 | Material                   | Brinell hardness |         |         |
|----|----------------------------|------------------|---------|---------|
|    |                            | 70° F.           | 350° F. | 450° F. |
|    | Hard babbitt*              | 33.9             | -----   | 3.6     |
|    | Cadmium 93.6%, silver 6.4% | 39.1             | 10.9    | 6.3     |
|    | Cadmium 92.0%, silver 8.0% | 47.2             | 11.4    | 6.3     |
|    | Cadmium 90.7%, silver 9.3% | 53.0             | -----   |         |

\*85% tin, 7.5% copper, 7.5% antimony.

It will be observed that the hardness of the softer of the two cadmium-silver alloys is somewhat greater than this particular hard babbitt at a temperature of 70° F. It is also evident that increasing the silver content of these alloys increases the hardness. Alloys softer than these can be obtained by using lower silver, and harder alloys by using higher silver content. It will be noted that at the temperature of 450° F. the cadmium-silver alloys are much harder than the babbitt and that the babbitt is very low in hardness at this temperature. Since the electrode-

posited alloys have very fine structures, it is believed that their hardness will be at least as great as in the as-cast alloys of similar compositions.

In order to compare further the properties of the cadmium-silver alloys with babbitt, pounding tests have been made. It is known that in bearing service the bearing linings are subjected to more or less of a pounding action and that some of them fail because of low resistance to pounding. The following table shows the results of tests on two cadmium-silver alloys in the cast condition and on three babbitts also in the cast condition. The results have been reported in terms of the number of blows required to deform cylindrical specimens (1 cm. in diameter and 2 cm. in height) 5 per cent of their height, using a hammer weighing 7.15 pounds which was permitted to fall through a height of two inches. The results in all cases are 20 the averages of two tests.

25 *Pounding tests on cadmium-silver alloys and on babbitts\**

| Material             | Composition                | Blows to deform 5% |
|----------------------|----------------------------|--------------------|
| Cadmium-silver alloy | 93.6% Cd, 6.4% Ag          | 70                 |
| Cadmium-silver alloy | 92.0% Cd, 8.0% Ag          | 125                |
| Babbitt              | 90.0% Sn, 4.5% Cu, 4.5% Sb | 12                 |
| Babbitt              | 87.5% Sn, 4.0% Cu, 7.5% Sb | 14                 |
| Babbitt              | 83.8% Sn, 7.5% Cu, 7.5% Sb | 33                 |

30 \*Tests with 7.15-lb. hammer falling 2 in.

The data show that even the softer of the two cadmium-silver alloys containing only 6.4% silver required 70 blows to deform it 5 per cent, whereas the hardest of the babbitts required only 33 blows to deform it 5 per cent. These results show that the resistance to deformation in pounding is increased as the silver content of these alloys is increased. Thus, if I wish to use an alloy to have high conformability I use an alloy lower in silver content, and if I wish to have an alloy of high hardness and high resistance to pounding I use an alloy of higher silver content.

These alloys, both cast and electrodeposited, on steel, cast iron, copper and bronze, have been subjected to wear tests and to actual bearing tests. In tests with the Amsler wear testing machine, an alloy containing 6.4 per cent of silver was found to give good performance. This was also true of a specimen containing 8.0 per cent of silver. When tested at as high a pressure as 3,250 lbs. per sq. in., the bearings performed satisfactorily without excessive wear and without wiping or seizing on the steel shaft on which they were run in contact. Babbitts in a similar test usually fall at pressures of 2,000 to 3,000 lbs. per sq. in.

The most conclusive test to which these bearing linings have been subjected comprises using them in connecting rods in an automotive engine under very severe service. These bearing linings, formed by electrodeposition, were applied to backs of argentiferous copper, the lining being only 0.004 to 0.005 in. in thickness. In one series of tests three connecting rod bearings lined with alloys containing 11.7, 11.0 and 5.6 per cent of silver were used. These bearings were run-in by starting the engine without a load at relatively low speed, gradually increasing the speed to about 3,000 R. P. M. over a period of about 30 hours. Afterwards, these bearings were subjected to the test which consisted of loading the engine and running it at full throttle at about 3,100 R. P. M. for a total period of 30 hours. The bearings 75

were then examined. The alloy containing 5.6 per cent of silver showed more wear, indicating that such an alloy is somewhat soft for this service. On the other hand, the alloys containing 5 11-12 per cent of silver had given very good performance. One of these alloys was continued in an additional run of 50 hours with the motor loaded and operating at full speed. Two other bearings containing 7.5 per cent of silver were 10 run in the second test, which consisted of running-in the bearings as described above and then running 50 hours at full throttle under load. Three commercial babbitt bearings were run for comparison. The advantages noted in the cadmium-silver alloys may be listed as follows:

Lower rate of wear was observed in the cadmium-silver linings. Cadmium-silver alloy linings containing 7.5 per cent of silver, after running 30 hours for running-in and 50 hours with 20 the engine loaded while operating at full throttle, showed practically no wear. They had bright polished surfaces when removed from the engine, whereas babbitt bearings used in the engine at the same time and for the same periods were dark 25 and coated, as well as being materially pitted. As other advantages of the cadmium-silver alloys, I have noted that they do not, within the range studied, show the tendency to flow under operating conditions, which I have observed in the 30 babbitt bearings.

I find that alloys containing from about 3 per cent to about 12 per cent of silver by weight have good bearing properties, in such service as bearing linings for connecting rods in an automotive engine. I consider, however, that in this particular service an alloy containing from 7 to 8 per cent of silver has somewhat better bearing properties than alloys having 5 per cent silver content or 12 35 per cent silver content.

It should be understood that my invention is not limited to the formation of binary alloys for bearing alloy material. More than two metals may be alloyed and, as long as silver and cadmium are embodied in the alloy, with cadmium the 40 principal constituent and constituting at least 80 per cent by weight of the alloy, such alloy will be within the scope of my invention. Likewise, it is not necessary that the small hard particles which are dispersed throughout the matrix be formed 45 by the use of an excess of silver over and above that amount which enters into solid solution with the cadmium. For example, it is within the scope 50 of my invention to utilize a metal or metals, in addition to the cadmium and silver, which will form small hard particles in the nature of intermetallic compounds either with the cadmium or the silver or with both. Metals answering this 55 description include copper, arsenic, nickel, zinc, magnesium, antimony and tin, though tin has certain undesirable properties which may render its use undesirable. One or more of these metals 60 may be used in percentages preferably, though not necessarily, smaller than the percentage of silver used. When using these minor amounts of other compound-forming elements to produce the hard particles, I may correspondingly reduce the silver 65 content, but the silver content should be kept sufficient to preserve the desired properties of the matrix.

It will be seen from above that I have devised 70 an alloy for bearing lining material embodying a matrix formed primarily of cadmium, with silver in solid solution therein whereby this matrix is rendered relatively tough while retaining the desired degree of hardness. In the preferred form

of my alloy, small hard particles are dispersed throughout this matrix, preferably in the form of intermetallic compounds which serve to make the contact and directly carry the load without impairing the conformability of the matrix.

It is also of importance that the alloy which I have produced has a higher melting point than the babbitt alloys. Likewise, the tests above referred to show that the alloy possesses a resistance to deformation by pounding which is far superior 10 to the babbitt alloys.

As already pointed out, the addition of silver to the cadmium improves the casting quality of the cadmium and makes it less susceptible to oxidation. Thus, the tendency of the cadmium to 15 dross is overcome very materially. Likewise, the silver improves the structure and physical characteristics of the alloy, imparting strength and hardness thereto. The silver not only increases 20 the fluidity of the alloy with a consequent improvement in casting qualities as indicated, but it even raises the melting point slightly.

Thus, I have been able to produce a bearing alloy with a base of cadmium, with its higher melting point and greater hardness than tin or 25 lead and have imparted strength, hardness and toughness by the addition of silver which, at the same time, improves the casting qualities of the 30 alloy. Likewise, whether my alloy be a binary alloy or whether it be formed of more than two 35 elements, I have introduced the additional metal or metals into the cadmium in sufficient proportion to bring about dispersion of small hard particles of intermetallic compound throughout the matrix which is preferably formed by the solid 40 solution of the silver and the cadmium.

Having thus described my invention, what I claim is:

1. A bearing material comprising essentially a 40 matrix consisting of cadmium with silver in solid solution therein, in combination with small hard particles of an intermetallic compound including one of said elements dispersed throughout said matrix, the silver being present in an appreciable amount not exceeding 15 per cent by weight of 45 the balance of the metal in the alloy.

2. A bearing alloy comprising a cadmium-rich cadmium-silver matrix, with the silver not exceeding 15 per cent of the total metal of the alloy, and a multiplicity of small hard particles of an 50 intermetallic compound including one of said elements dispersed throughout said matrix.

3. A bearing alloy comprising a cadmium base with a silver content not exceeding 15 per cent 55 of the total metal of the alloy and being in excess of that amount which will enter into solid solution in the cadmium whereby there is formed a matrix of cadmium with silver in solid solution therein and a multiplicity of small hard particles of an intermetallic compound of cadmium and 60 silver.

4. A bearing alloy comprising from .10 to 15 per cent of silver and the balance substantially cadmium.

5. A bearing alloy consisting of from 3 to 15 per 65 cent of silver and the balance substantially all cadmium.

6. A bearing alloy consisting of cadmium and silver, with the silver 5 to 12 per cent by weight of the total and with the remainder substantially 70 all cadmium.

7. A bearing alloy comprising a relatively soft matrix formed primarily of cadmium with silver in solid solution therein and a multiplicity of small hard particles primarily of a silver-cad- 75

mium compound dispersed throughout said matrix, the silver in said alloy being from substantially about 3 to 15 per cent by weight and the balance of the alloy being primarily of cadmium.

- 5 8. A bearing alloy comprising a matrix consisting of cadmium with silver in solid solution therein, said matrix having small hard particles of an intermetallic compound including one of said elements dispersed therethrough, the silver being present in an amount not less than 3 per cent and not exceeding 15 per cent by weight of the balance of cadmium in the alloy.
- 10

9. A bearing alloy comprising a matrix consisting of cadmium with silver in solid solution therein, said matrix having small hard particles of an intermetallic compound including one of said elements dispersed therethrough, the silver being present in an amount not less than .10 per cent and not exceeding 15 per cent by weight of the balance of cadmium in the alloy. 5

10. A bearing alloy comprising from .5 to 5% of silver and the balance substantially cadmium. 10

OSCAR E. HARDER.